

March 30, 1926.

1,578,688

E. A. SPIES

PLASTER OF PARIS BANDAGE

Filed Sept. 24, 1924



WITNESSES  
J. Apfel  
Geo. Ocker

INVENTOR  
EDWIN A. SPIES

BY  
T. Burns  
ATTORNEY

Patented Mar. 30, 1926.

1,578,688

# UNITED STATES PATENT OFFICE.

EDWIN A. SPIES, OF PELHAM, NEW YORK.

## PLASTER-OF-PARIS BANDAGE.

Application filed September 24, 1924. Serial No. 739,622.

*To all whom it may concern:*

Be it known that I, EDWIN A. SPIES, M. D., a citizen of the United States, and a resident of Pelham, in the county of West-  
5 chester and State of New York, have invented a new and Improved Plaster-of-Paris Bandage, of which the following is a full, clear, and exact description.

This invention relates to a plaster of Paris 10 bandage and has for an object the provision of an improved bandage for use in surgical practice to support or restrain various mobile portions of the human anatomy.

More specific objects of the invention are 15 to provide a bandage economical to manufacture commercially, easy for the surgeon to apply and one which will provide the patient with proper support combined with maximum comfort.

20 With such objects in view and others which will appear as the description proceeds, the invention comprises novel features of construction which will be set forth with particularity in the following description and claims appended hereto.

In the accompanying drawing which 25 illustrates one embodiment of the invention, Fig. 1 is a somewhat magnified section of the cloth used in the construction of this bandage. This is a thin, loosely woven cotton cloth, gauze or scrim sized with starch or some other sizing or stiffening agent, of about 28/32 to 42/48 mesh, weighing about 30 2½ ounces per square yard, and prepared in standard widths of the number of inches desired for the finished bandages. Fig. 2 is a partial view of the completed bandage.

35 Referring to the drawing, the basic cloth 1 is woven without a selvage by having the 40 transverse fibers or threads (2) woven in one continuous piece, each of which turns about and around the ultimate longitudinal fibers or threads (3) so that said longitudinal threads will be held in their respective 45 places and prevented from becoming dislodged and thereby separated from the body of the cloth. Or the cloth may be made in standard widths with a narrow selvage (4) of from two to six threads on each margin and also with a series of longitudinal close weavings (5) of from two to six threads at regular intervals across the width 50 of the cloth. Or it may be made in standard widths with any other similar weave for the 55 aforementioned purpose, sized in the above manner, producing a bandage cloth whose

ultimate marginal longitudinal thread or threads cannot separate from the body of the cloth during handling, and whose elongation characteristics are uniform throughout its entire width.

At (6) I show a thin layer of dry plaster of Paris which has been ground, rubbed or otherwise forced into the meshes of the cloth so as to constitute a uniformly distributed 65 amount of plaster throughout the bandage, amounting by weight to about 6¾ ounces per square yard of cloth. At (7) I show the layers of cloth wound into the completed bandage and ready for the surgeon. The 70 bandage is wound at a particular tension, amounting to about 1½ to 2½ ounces per inch width of cloth. I make the core (8) approximately 1" in diameter.

75 Due to the particular cloth used, I produce a bandage free from loose marginal longitudinal threads which make the bandage exceedingly difficult to handle and are a frequent cause of embarrassment to the operating surgeon. The loose threads also afford 80 a difficulty in the making of plaster splints in that their attempted removal ordinarily causes the windings of the bandage to become wrinkled producing extreme discomfort to the patient when the splint is dry 85 and moreover they add to the difficulty of properly moulding the splint to the anatomical part.

90 Due to the uniform layer of plaster thoroughly pressed into the cloth I avoid the non-water-permeable characteristics of the bandage with too much plaster, the non-adhesive properties of the bandage with too little plaster, and the lumpy and uncomfortable effect of the bandage combining both 95 defects.

95 Due to the particular tension of my bandage in the dry state, I attain the proper degree of water saturation and avoid washing away of the plaster.

100 Due to the large core hole in my bandage I allow a sufficient quantity of water to enter and attack the layers from within outward during the immersion process thereby avoiding an inequality of saturation.

105 Having described the nature of my invention, I claim as new and desire to protect by Letters Patent:—

110 1. A plaster of Paris bandage adapted to be formed into an efficient, comfortable, neat appearing and easily constructed anatomical support for various portions of the

human body, comprising, in combination, a loosely woven non-selvage cotton cloth or gauze of 28/32 to 42/48 mesh sized with starch or glue and weighing 2 to 3 ounces per square yard, a uniformly distributed layer of dry plaster of Paris amounting to 6 to 7 ounces per square yard of cloth and the cloth and plaster being wound into a completed roll with a tension of 1 to 3 ounces per inch width of cloth with a core hole approximately 1" in diameter.

2. A plaster of Paris bandage adapted to be formed into an anatomical support, comprising a loosely woven cotton cloth or gauze of 28/32 to 42/48 mesh sized with starch or glue weighing 2½ ounces per square yard manufactured in standard widths of the number of inches desired for the finished bandages and a uniformly distributed filler of plaster of Paris.

3. A plaster of Paris bandage comprising a loosely woven cloth without selvage, with longitudinal close weavings of from 2 to 6 threads at regular intervals across the width of the cloth and a uniformly distributed 25 layer of dry plaster of Paris amounting by weight to 6¾ ounces per square yard of cloth.

4. A plaster of Paris bandage comprising a carrying cloth over which has been deposited a uniform layer of dry plaster of Paris, the cloth and plaster being wound into a completed roll with a tension of 1½ to 2½ ounces per inch width of cloth.

5. A plaster of Paris bandage comprising alternate layers of carrying cloth and dry plaster of Paris, and a core hole 1" in diameter.

EDWIN A. SPIES, M. D.